

## 1

3,027,254

**NICKEL-COBALT BASE ALLOYS**

Jerome Benedict Mulerich, West Peabody, and Robert Francis Wilde, Lynnfield, Mass., assignors to General Electric Company, a corporation of New York  
 No Drawing. Filed Apr. 21, 1959, Ser. No. 807,789  
 3 Claims. (Cl. 75—171)

This invention relates to nickel-cobalt base alloys suitable for casting, particularly unique in improved elevated temperature ductility and impact strength.

Designers of articles intended for use at elevated temperatures under stress and vibratory conditions resist the use of materials having low ductility and poor resistance to impact. Unfortunately, the properties of many cast materials include such undesirable properties, yet the production costs of many articles manufactured by casting methods, such as accurate vacuum investment casting methods, are considerably lower than other methods such as machining or forging.

Therefore a principal object of our invention is to provide a casting alloy having suitable strength characteristics for elevated temperature applications under stress conditions and including greater ductility and impact strength properties than currently available cast alloys.

Another object is to provide a nickel-cobalt alloy including a balance of aluminum, titanium, carbon, molybdenum and iron to provide ductility in a casting usually found in wrought articles.

Our alloy in one form comprises in percent by weight about 0.10–0.16 carbon, about 2–2.5 titanium, about 3.5–4 aluminum, about 4–5 molybdenum, about 14–16 chromium, about 26–28 cobalt, up to about 2 iron, about .01–.02 boron, with the balance essentially nickel, impurities, and the usual small quantities of manganese and silicon. However, we prefer that our alloy include in percent by weight a maximum of about 0.2 manganese and a maximum of about 0.3 silicon.

Our alloy features excellent ductility and impact strength principally as a result of a balance between the alloying of titanium, aluminum, iron, molybdenum and carbon with a nickel-cobalt base including chromium. We have found that the ductility and impact strength is maintained at a superior level if the Al/Ti ratio is at about 2 or below, at the same time as the Ti/C ratio is maintained at about 16 or below and the Mo/Fe ratio is about 2.5 or greater.

We prefer to refer to our alloy as a casting alloy because it displays excellent stress rupture strength inherent in castings over that of wrought materials. For example, in the range of about  $\frac{1}{64}$ "– $\frac{1}{16}$ " our alloy exhibits average 100 hours stress rupture life at 1350° F. of 68,000 pounds per square inch, at 1500° F. of 46,000 pounds per square inch and at 1650° F. of 28,000 pounds per square inch. However our alloy has the ductility for engineering applications generally only obtainable in wrought materials.

In order to determine the ductility, sometimes referred to as "tensile ductility," of our alloy in its broad range, we conducted a series of tensile tests from which may be calculated the "ultimate tensile strength," referred to in the tables as "U.T.S.," "percent elongation" and "percent reduction in area." "Ultimate tensile strength" is the value in pounds per square inch obtained when the maximum load recorded during the straining of a specimen is divided by the cross sectional area of the specimen before straining. "Tensile ductility" is the measure of the permanent deformation before fracture by stress when the specimen is in tension. "Percent elongation" may be defined as the amount of permanent extension in the vicinity of the fracture during a tensile test expressed as percentage of the originally gage length; the "percentage reduction in area," shown as "percent R.A." in the tables, may be de-

## 2

fined as the percentage difference between the original cross sectional area and that of the smallest area at the point of rupture of a test specimen.

Table I represents average and maximum tensile data for a large number of specimens tested having grains sizes up to about  $\frac{1}{16}$ ". Our alloy was cast directly into the 0.250 inch diameter test specimens size and had a grain size range of about  $\frac{1}{64}$  to  $\frac{1}{16}$  inch. The gauge length of the test specimens upon which the following elongation values were based was 1 inch.

Table I

| Temp. (° F.) | U.T.S. (1,000 p.s.i.) |      | Elongation (percent) |      | R.A. (percent) |      |
|--------------|-----------------------|------|----------------------|------|----------------|------|
|              | Avg.                  | Max. | Avg.                 | Max. | Avg.           | Max. |
| Room         | 148                   | 158  | 6                    | 10   | 6              | 9    |
| 1,200        | 132                   | 150  | 7                    | 14   | 13             | 23   |
| 1,500        | 113                   | 126  | 3                    | 5    | 7              | 13   |

Another measure of ductility of an alloy is an impact test conducted to determine the energy, usually measured in foot pounds, absorbed in fracturing a test bar. The impact test which we used was a standard A.S.T.M. V notch Charpy impact test performed on a test bar cantilevered at both ends and including a notch in one face. The bar is impacted on the side opposite the notch by a falling weight possessing a potential energy of about 117 foot pounds. We obtained the average data shown in Table II from alloys having the composition in percent by weight of 0.10–0.16 carbon, 2–2.5 titanium, 3.5–4.0 aluminum, 4–5 molybdenum, 14–16 chromium, 26–28 cobalt, a maximum each of 0.2 manganese and 0.3 silicon, a maximum of 2 iron, 0.01–0.02 boron with the balance essentially nickel and impurities (grain size= $\frac{1}{16}$ "':

Table II

| Temp. (° F.): | Impact force (foot pounds) |
|---------------|----------------------------|
| Room          | 7                          |
| 1200          | 8                          |
| 1500          | 12                         |
| 1700          | 20                         |

Although a number of cast nickel base alloys have been reported as suitable for elevated temperature applications, we have found it to be desirable to maintain our Al/Ti ratio at or below about 2 at the same time as our Ti/C ratio is at or below about 16 and our Mo/Fe ratio is at least at about 2.5 within the range of our alloy.

Table III compares these essential elements in some other cast alloys, the impact strengths of which we tested with our alloy.

Table III

|       | Our Alloy | Alloy A   | Alloy B |
|-------|-----------|-----------|---------|
| Al    | 3.5–4.0   | 4.5       | 3       |
| Ti    | 2–2.5     | 3.5       | 3       |
| C     | 0.1–2     | 0.08 max. | 0.1     |
| Mo    | 3.5–5     | 5.5       | 4       |
| Fe    | 0.1–2     | 5         | 2       |
| Al/Ti | 2 max.    | 1.3       | 1       |
| Ti/C  | 16 max.   | 43        | 30      |
| Mo/Fe | 2.5 min.  | 1.1       | 2       |

Table IV gives the results of impact testing at 1500° F. using the Charpy V notch impact test (grain size= $\frac{1}{16}$ "':

Table IV

| Alloy: | Impact force (foot pounds) |
|--------|----------------------------|
| Our    | 12                         |
| A      | 4                          |
| B      | 10                         |

Although we have described our alloy in connection

with specific examples referring to grain size in a certain range and our alloy tested in the as-cast condition, it will be understood by those familiar with the art of metallurgy and heat treatment the variations and modifications of which our alloy is capable.

What we claim is:

1. A nickel-cobalt base cast alloy comprising in percent by weight about 0.10-0.16 carbon, about 2-2.5 titanium, about 3.5-4.0 aluminum, about 4-5 molybdenum, about 14-16 chromium, about 26-28 cobalt, up to about 2 iron, about 0.01-0.02 boron, with the balance essentially nickel and impurities and having an Al/Ti ratio of about 2 or below, a Ti/C ratio of about 16 or below and Mo/Fe of at least about 2.5.

2. An article cast from the alloy of claim 1 having a grain structure in size up to about  $\frac{1}{16}$ ".

3. A nickel-cobalt base cast alloy comprising in per-

cent by weight about 0.10-0.16 carbon, about 2-2.5 titanium, about 3.5-4.0 aluminum, about 4-5 molybdenum, about 14-16 chromium, about 26-28 cobalt, up to about 2 iron, about 0.01-0.02 boron, a maximum each of about 0.2 manganese and about 0.3 silicon with the balance essentially nickel and impurities and having an Al/Ti ratio of about 2 or below, a Ti/C ratio of about 16 or below and Mo/Fe ratio of at least about 2.5.

10

References Cited in the file of this patent

UNITED STATES PATENTS

2,688,536 Callaway et al. ----- Sept. 7, 1954

FOREIGN PATENTS

548,778 Canada ----- Nov. 12, 1957  
92,627 Norway ----- Oct. 13, 1958

15